

July 31, 1923.

1,463,771

A. A. CLAASSEN

MEANS TO COMPRESS INGOTS

Filed April 17, 1922



Fig. 4.



Fig. 5.



Witness:

Richard J. Jackson

Inventor:

A. A. Claassen

*By J. M. Roberts*

*This 31st day of July, 1923.*

Patented July 31, 1923.

1,463,771

# UNITED STATES PATENT OFFICE.

ALVIN A. CLAASSEN, OF CHICAGO, ILLINOIS.

## MEANS TO COMPRESS INGOTS.

Application filed April 17, 1922. Serial No. 553,694.

To all whom it may concern:

Be it known that I, ALVIN A. CLAASSEN, a citizen of the United States, residing at Chicago, in the county of Cook, State of Illinois, having invented certain new and useful Improvements in Means to Compress Ingots, do hereby declare that the following is a full, clear, and exact description thereof, such as will enable others skilled in the art 10 of making steel to practice the same.

In the manufacture of castings or ingots as the molten metal cools in the mold or jacket gas-pockets and internal shrinkage cavities and pipes form in the upper portion 15 of the solidifying mass, and also segregations of material occur as some of the constituents of the steel, such as carbon and certain impurities, tend to separate from the mass and gather toward the center or longitudinal axis of the ingot as it cools. These 20 factors unfavorably affect the properties of the metal and develop imperfections in the product.

The object of my present invention is to 25 provide new and improved means to reduce the formation of gas-spaces and pipes and the occurrence of these segregations, and it consists in simple and efficient devices of the character hereinafter pointed out for laterally bending or compressing the upper 30 portions of the solidifying sides of the metal in the mold between its corners inwardly toward the center of the mass.

A practical embodiment of my invention 35 is shown in the accompanying drawing, in which Fig. 1 is a top plan view of a mold equipped with compression bars on its sides between its corners; Fig. 2 is a longitudinal sectional view of the same on the line 2—2 40 in Fig. 1; Fig. 3 is a view similar to Fig. 2, but taken at a right angle thereto and with the keys of the compression bars removed and wedges in place in the mold; Fig. 4 is a detail cross-sectional view of one of the compression bars on the line 4—4 in Fig. 2, and Fig. 5 shows a modification.

In the use of my invention the casting operation is carried out in the usual manner, and in the drawing the reference numeral 1 50 indicates the body of an ingot mold or jacket which is of usual size and configuration, and has the usual ears 2 at its upper end. The mold is provided with a plurality of compression bars 3 of cast steel, which are 55 rectangular in shape, and are of sufficient length to extend into the mold approxi-

mately to a depth of about half its length, and of sufficient width to cover approximately a third of the width of the inner faces of the sides of the mold; the only 60 essential as to their width is that they leave a margin at each side so that the corners of the mold are not covered. The number of bars employed varies with the cross-sectional shape of the mold, that shown in the 65 drawings being square and equipped with four bars, one at the center of each side as shown in Fig. 1. The bars are suitably supported on the mold so as to be movable inwardly toward its center. In the form 70 shown each bar has its upper end shaped into a hook 4 to take over the upper edge of the mold and longer than the thickness of the material of the mold so that the upper end of the bar is free to move inwardly, and 75 the body of each bar is provided with a pair of spaced upper and lower pins 5 and 6, respectively, constructed to extend outwardly through upper and lower slots 7 and 8, respectively, in the sides of the mold, the upper pins and slots being positioned a few 80 inches below the top end of the mold and the lower ones a few inches above the center of its longitudinal axis or length. The bars are held in position tight against the faces 85 of the mold during the pouring of the metal and partial cooling of its outer portion by wedge-keys or gibs 9 passing through holes 10 in the outer portions of their pins. After 90 the metal is tapped-off into the mold and its outer portion has cooled or solidified sufficiently to form a flexible crust or skin, the keys are released by partly or wholly withdrawing them from the pins, and the bars are moved inwardly to compress or bend the 95 upper portions of the centers of the sides of the metal between its corners toward its center. This compression movement of the bars may be accomplished by any suitable means; in the form shown for this purpose the bars 100 are provided on their outer faces with elongated open-top slots or troughs 11 extending through their upper hooked ends and to a point near their lower ends, and preferably tapered from top to bottom in the cross-sectional line of the adjacent wall, to receive correspondingly tapered wedges 12 which are constructed so that as they are driven into place between the bars and the face of the mold they will crowd or move the 105 bars inwardly toward the center of the ingot. The wedges are relatively thickened

toward their upper ends; in practice they are about an inch and one-half thick at the top and gradually diminish to the bottom so that they move the bars inwardly with more or less of a pivotal motion on their lower feet 13 to increase the compression toward their upper ends.

By this arrangement the bars are initially held tight against the face of the mold so that no metal will pass behind them, and after the outer portion of the metal has solidified sufficiently to form a flexible crust, which usually occurs in ten minutes after it is poured, the keys are released and the wedges are driven into place, and the compression bars are moved inwardly to compress or bend the upper parts of the ingot between its corners toward its center. The condensation and pressure produced by this lateral inward bending or compression eliminates segregation and the formation of pipe and gas-holes and forces the CO gas up to the top of the ingot where it passes out. As the segregation, piping and gas-holes occur in the upper portion of the ingots during their cooling or solidification in the molds, and increasingly toward their upper ends, the inward compression of the upper part of the ingot during its solidification in the mold is particularly effective in eliminating these objections without affecting the other portions of the ingot. The inward movement of the bars to bend the ends of the sides of the ingot about a quarter ( $\frac{1}{4}$ ) or half ( $\frac{1}{2}$ ) an inch is sufficient for high carbon steel, and will be greater for softer steels.

Processes have been previously proposed for compressing a cooling ingot involving among others the steps of raising and lengthwise compressing it against a solid ram or abutment above it; also of forcing the ingot upward into its tapered mold during solidification, and also of stripping the ingot from its mold and running it on its car between a solid and a movable wall which latter is then pressed against one side of the ingot, but practice has shown that these methods do not either reduce or remove the known objections and disadvantages, and in some instances produce others that also are detrimental to the properties of the metal.

By my invention these former objections of segregation, piping and gas-holes are practically eliminated, the castings are solid substantially throughout and the amount

wasted by cropping is negligible, and the original composition and properties of the metal are not materially affected.

The mold may have recesses 14 in its inner faces for the bars 3 as shown in Fig. 5.

I claim:

1. An ingot mold, a plurality of compression bars constructed to extend into the upper end of the mold and to cover the central portions of its sides, releasable means to hold the bars tight against the sides of the mold, and wedges constructed to be driven between the mold and bars to move the bars inwardly toward the center of the mold when their holding-means are released. 65

2. An ingot mold having spaced upper and lower slots in its sides, a plurality of compression bars constructed to extend into the upper end of the mold and to cover the central portions of its sides, pins on the bars constructed to pass through said slots, keys constructed to removably engage the outer ends of the pins to hold the bars tight against the sides of the mold, and means to move the bars inwardly toward the center of the mold when their keys are released. 75

3. An ingot mold having spaced upper and lower slots in their sides, a plurality of compression bars constructed to extend into the upper end of the mold and to cover the central portions of its sides, pins on the bars constructed to pass through slots, keys constructed to removably engage the outer ends of the pins to hold the bars tight against the sides of the mold, and wedges constructed to be driven between the mold and bars to move the later inwardly toward the center of the mold when their keys are released. 85

4. An ingot mold having spaced upper and lower slots in its sides, a plurality of compression bars constructed to extend into the upper end of the mold and to cover the central portions of its sides, each bar having an open-top slot extending from its top to near its lower end, pins on the bars constructed to pass through the slots of the mold, keys constructed to removably engage the pins to hold the bars tight against the sides of the mold, and wedges constructed to enter the slots in the bars and move the latter inwardly toward the center of the mold when their keys are released. 100

In testimony whereof I hereto affix my signature.

ALVIN A. CLAASSEN.